

(No Model.)

L. E. OSBORNE.

FIRE KINDLER.

No. 329,070.

Patented Oct. 27, 1885.



WITNESSES

Geo. E. Scott

Harry N. Colburn

INVENTOR

L. E. Osborne

# UNITED STATES PATENT OFFICE.

LEONARD E. OSBORNE, OF LEOMINSTER, MASSACHUSETTS.

## FIRE-KINDLER.

SPECIFICATION forming part of Letters Patent No. 329,070, dated October 27, 1885.

Application filed December 4, 1884. Renewed September 19, 1885. Serial No. 177,570. (No specimens.)

*To all whom it may concern:*

Be it known that I, LEONARD E. OSBORNE, a citizen of the United States, residing at Leominster, in the county of Worcester and Commonwealth of Massachusetts, have invented 5 a new and useful compound to be used for kindling fires, of which the following is a specification.

My invention relates to that class of 10 pounds which are indestructible by fire, and used for the purpose of kindling fires, and is composed of the following ingredients, viz: hard-pan fire-brick clay, coarse mortar-sand, and hard white-ash coal. This forms a hard 15 block, when properly made, which is very porous and will endure any amount of heat, and may be used for an indefinite length of time.

To enable others skilled in the art to make 20 and use my invention, I will proceed to describe the proportions, manner of compounding, manufacturing, and using the same.

The accompanying drawing shows a sectional and end view of the fire-kindler.

25 First take of the first-named article, hard-pan fire-brick clay, two parts; second, take of coarse mortar-sand, one part; third, of hard white-ash coal, one-sixteenth part—all to be well pulverized and mixed together dry, 30 and then mixed with water to about the consistency of common mortar for plastering; fourth, put it in form by the use of molds, which may be of the desired length and widths.

The size I have adopted for a convenient 35 kindler is four inches long by one and one-fourth inch square. They may be made of larger sizes, when desired, to absorb more oil and burn longer. After being molded into shape they are placed in a position to dry 40 thoroughly in the open air. Then they are placed in a kiln or oven and burned two or three days, and when perfectly cooled they are ready for use. Now put them into a tin 45 box, or any tight vessel, and cover them with kerosene-oil, allow them to remain in the oil a short time, until perfectly saturated. Then when a match is applied they readily 50 ignite and produce a volume of fire that will burn fifteen or twenty minutes, which will kindle any dry-wood or soft-coal fire. When the fire is sufficiently low, take them out and properly cool and put them into the oil again for a few minutes, or until wanted for use again.

Having thus described my invention, what 55 I claim as new, and desire to secure by Letters Patent, is—

A compound, as herein described, for a fire-kindler, prepared from and consisting of hard-pan fire-brick clay, hard white-ash coal, and 60 coarse sand, in the manner and for the purpose specified.

LEONARD E. OSBORNE.

Witnesses:

CHARLES WILD,  
C. W. CARTER.